

Feb. 8, 1949.

J. GOMBOSH

2,461,052

METHOD OF CASTING

Filed Oct. 21, 1944

*Fig.1.*



*Fig.2.*



INVENTOR

John Gombosh  
by his attorney  
Christy, Pamelos & Stukel

## UNITED STATES PATENT OFFICE

2,461,052

## METHOD OF CASTING

John Gombosh, Pittsburgh, Pa.

Application October 21, 1944, Serial No. 559,763

4 Claims. (Cl. 22—209)

1

This invention relates to metal founding, and more particularly the casting of large metal bodies such, for example, as rolling mill rolls, ingots, and other large bodies where piping has heretofore been a detrimental factor.

In the casting of large bodies of metal, it is well known that the outside solidifies before the center, and that portions of small sections usually solidify before portions of large section. The solidification of the exterior of the body followed by the cooling and shrinking of the molten interior, results in the formation of a cavity or pipe in the upper end of the casting which may extend an indeterminate depth into the body of the metal. Moreover, the solidification of the metal may be such as to set up strains, especially in the casting of objects such as rolling mill rolls, tending to cause the neck of the roll to break at a point intermediate its length. This breakage is usually manifested by a convex surface on the stump of the roll neck that remains attached to the roll body.

The present invention provides a mold and a method of casting which substantially reduces, and to a large extent, eliminates such conditions. The invention contemplates a method of procedure in which the mold is filled with hot metal to a point of overflowing, whereby dross and impurities that often float on the top of the metal are floated outside of the mold cavity. After the mold has been filled to this extent, a separating disc is placed in position on top of the molten metal and then further metal is floated into means providing a reservoir in the upper part of the mold cavity. The function of the reservoir is firstly, to provide a body of hot metal that will retard the cooling of the upper part of the casting, and secondly, to cover the disc and provide a pressure downwardly against the disc. If a pipe tends to form, it forms first in this auxiliary body of metal. It may extend down to the disc, and there it will be interrupted by the disc, and can extend no lower. As shrinkage of the metal occurs under the surface of the disc, the disc will move or be pressed down and to some extent, hot metal above the disc may flow around its edges to the body of the casting below. Whatever the exact mechanism, the disc or separator serves to eliminate pipe below it.

The invention may be more fully understood by reference to the accompanying drawings, in which:

Fig. 1 represents a longitudinal, vertical section through a mold for casting a rolling mill roll, said mold embodying my invention; and

Fig. 2 shows the application of my invention to a conventional ingot mold which may be either a bottom pour or a top pour mold, but is preferably a bottom pour mold.

Referring first to the drawings, 2 designates

2

a sand mold contained within a suitable casing not shown, and which has a cavity 3 conforming to the roll to be cast. At the lower end is a portion 4 forming a neck at one end of the roll. At the top of the cavity 3 there is a built-up extension 5 to form the other neck of the roll, this extension 5 being spaced from the exterior of the mold body, thereby providing an annular trough 6 around the extension 5, the body 2 of the mold projecting a substantial distance above the extension 5. The extension 5 is preferably tapered exteriorly toward its base.

In using the mold, hot metal is poured in the usual manner into the mold cavity through the top thereof until the extension 5 has been filled, and the pouring is then continued to float the dross and impurities over the top of the extension 5 into the annular trough 6. After this part of the process has been performed, a separating disc 7 of a size to loosely fit into the extension 5 is placed in the top of the extension. The separating disc may be either of metal or refractory, metal having a higher melting point than the metal in the mold preferably being used. The separator will preferably be such that tend to float on top of the molten metal in the extension 5, in which case heavy restraining elements 8 may be placed over the top of the plate, before the additional metal is added. If the plate is heavier, and in order to assure that the separator will not sink to the bottom, the interior of the upper part of the extension 5 may be countersunk and the separator be of a diameter such that should it sink, it could not pass below the shoulder 9 at the bottom of this enlarged or countersunk portion. It may be noted that in practice the cold metal separator, when placed flatwise on the molten metal, does not sink. After the disc is in place, more molten metal is poured into the top of the mold to completely fill the cavity 6 and cover the separator to a depth of several inches.

After this has been done, the casting is allowed to cool. The body of metal in the channel 6 keeps the narrow section of metal forming the upper roll neck hot, so that it does not solidify rapidly. The head of metal above the disc 7 presses down on the disc so that as shrinkage occurs in the casting comprising the roll, the disc moves down, tending to keep the end of the casting even. If a pipe starts to form, it will form in the metal above the disc 3 because the pipe forms from the outside of the molten mass toward its center. Any opening that thus tends to develop may reach the separator plate 7, but there can be no continuity of that opening below the separator. There will be no formation of any secondary pipe below the separator because of the downward pressure of the separator against the metal, and because the pipe starts at

the exterior and not internally. The disc 7 is sufficiently loose so that gases can escape around it, and so that molten metal may flow around the edges into the part of the cavity below the separator.

Fig. 2 illustrates the application of my invention to the casting of ingots wherein 10 designates a conventional ingot mold, preferably a bottom pour mold. Set into the upper portion of this mold below the top thereof is a frustoconical pressed metal shell 11 which may be either frictionally held in the mold cavity, or the mold cavity may be provided with a recess or shoulder for supporting it. It has an open center designated 12. As shown in Fig. 2, it is set into the mold cavity so that it slopes upwardly and inwardly.

In operation, hot metal is charged into the mold cavity until it overflows through the opening 12, allowing the dross and impurities to overflow into the annular trough 13 provided around the exterior of the body 11, and the interior of the mold. A separator plate 14 is then set in the hole 12 and more metal is poured into the top of the mold to a height of several inches above the separator.

Thus there is provided a condition similar to that described in connection with Fig. 1, in which there is an annular body of molten metal 13 around the upper part of the ingot with an overlying body of metal pressing down on the disc 14. Shrinkage which tends to occur below the separator 14 causes the separator to move downwardly, and there is a convex body of metal under the member 11, instead of a concave body which is usually present in a cooling ingot. The separator may be supported against premature sinking by means of lugs or hooks 15 formed on the edge of the separator, and which contact the top of the cone if the separator sinks too far, these hooks normally being sufficiently above the top of the disc to let it move down several inches. Preferably, the separator floats on the metal and is restrained in place by heavier or non-floating elements 15'.

From both of the embodiments herein described, it will be seen that the invention comprises a method and apparatus for casting wherein there is a hot body of metal above the principal part of the casting with an intervening separator, the overlying body of metal pressing down on the separator, and also providing a trough to retard the cooling of the upper part of the body of metal being cast. It will also be seen that in both embodiments which are merely typical of various embodiments of my invention, provision is made for the cleaning of the principal mold cavity of dross and impurities by overflowing them from the mold cavity before the separator plate is put into place. It will be understood that the metal poured in above the separator is cropped off the finished casting and reused as scrap. It may be pointed out that in Fig. 1 the mold is a sand mold and in Fig. 2 it is a metal mold. The invention is applicable to either sand or metal molds, the latter sometimes being designated "chill" molds, and the mold of Fig. 1 might therefore be of metal or the mold of Fig. 2 might be sand.

While I have illustrated and described certain specific embodiments of my invention, it will be understood that these are merely by way of illustration, and that various changes and modifications may be made within the contemplation of

my invention and under the scope of the following claims.

I claim:

1. The method of casting metal objects in a mold wherein the mold has a vertical depth greater than the depth of the object to be formed and has an annular trough adapted to surround the upper part of the body to be formed, which comprises filling the mold cavity to a point where dross and impurities overflow from the mold cavity into said annular trough, substantially covering the trough of the metal casting to the mold cavity with a separator plate and then filling molten metal into the top of the mold to fill the annular trough and cover the separator plate so as to provide a depth of molten metal above the separator plate.

2. The method of casting large metal bodies which comprises forming the top of the mold cavity in which the body is to be cast with a portion of reduced cross sectional area, the portion of reduced area being surrounded by a trough for receiving the metal, filling the mold cavity with molten metal and overflowing dross and impurities into said annular trough, interrupting the pouring operation and placing a separator plate on top of the cast metal in the mold cavity, and then filling the trough and the mold cavity above the separator plate with molten metal.

3. The method of casting large metal bodies which comprises forming the top of the mold cavity in which the body is to be cast with a portion of reduced cross sectional area, the portion of reduced area being surrounded by a trough for receiving the metal, filling the mold cavity with molten metal and overflowing dross and impurities into said annular trough, interrupting the pouring operation and placing a separator plate on top of the cast metal in the mold cavity, and then filling the trough and the mold cavity above the separator plate with molten metal, the separator plate being adapted to float on the molten metal.

4. The method of casting large metal bodies which comprises forming the top of the mold cavity in which the body is to be cast with a portion of reduced cross sectional area, the portion of reduced area being surrounded by a trough for receiving the metal, filling the mold cavity with molten metal and overflowing dross and impurities into said annular trough, interrupting the pouring operation and placing a separator plate on top of the cast metal in the mold cavity, and then filling the trough and the mold cavity above the separator plate with molten metal, the separator plate being adapted to float on the molten metal, and restraining the separator from floating to the top of the overlying body of metal.

JOHN GOMBOSH.

#### REFERENCES CITED

The following references are of record in the file of this patent:

#### UNITED STATES PATENTS

| Number    | Name     | Date          |
|-----------|----------|---------------|
| 1,204,270 | Greene   | Nov. 7, 1916  |
| 1,546,796 | Saunders | July 21, 1925 |
| 2,127,277 | Turner   | Aug. 16, 1938 |
| 2,148,583 | Rowe     | Feb. 28, 1939 |

#### FOREIGN PATENTS

| Number  | Country       | Date          |
|---------|---------------|---------------|
| 386,860 | Great Britain | Jan. 26, 1933 |
| 456,933 | Great Britain | Nov. 18, 1936 |